

## UNITED STATES PATENT OFFICE

1,949,911

## PHOTOGRAPHIC DEVELOPER

Fritz J. Hepner, Potsdam, Germany

No Drawing. Application November 8, 1927,  
Serial No. 232,002. In Germany December 15,  
1926

2 Claims. (Cl. 95—88)

This invention has reference to a photographic developer for so-called long-time-horizontal photographic development, and it is intended to devise means of producing very uniformly developed pictures and to avoid or minimize the occurrence of clouds and other disturbances. The invention is an improvement upon the utilization of bromine for the equalization of strong contrasts of light which is based upon the observation that in the developing of photographic negatives bromine is separated which is dissolved in the developing liquid and in this condition produces a retarding action upon the developing procedure. If the negative is allowed to remain in a reclining position or as horizontally as possible and without agitation in a highly diluted developing solution for a sufficient length of time, comparatively more bromine will be eliminated at the majority of the portions exposed to the light than at those portions of the negative which have been less subjected to the action of the light. These comparatively larger quantities of the bromine separated out in the more lighted portions and which are deposited there, have a retarding action, while the portion upon which the light has acted less, will be developed and finished more quickly, relatively speaking, because smaller amounts of bromine will be liberated at these places.

Now it has been ascertained that by using developers of the usual composition disturbing clouds or veils are liable to be formed with this kind of long-time-horizontal development, and fluctuations of temperature are of great influence, and the degree of dilution is of importance, and can only difficultly be determined in advance, particularly where there is lack of distilled water. Now it results from my investigations and experiments that these difficulties may be overcome and that it is possible to produce negatives exhibiting a harmony of shades such as has been impossible to produce heretofore by any other procedure according to the previous art, particularly in a simple and easy manner, by making use of developers of any usual composition, but containing no caustic alkali, salts or other additions containing or forming caustic alkali by hydrolysis or other decomposition procedures, in combination with the long-time-horizontal developing process and in concentrations that are much lower than those used for the customary tank or stand development. It has been shown that with such developers the most delicate degrees of shades contained in the negative may be brought out, and the positives are

free from halos and clouds and with the entire outlines of the picture in shadow parts. This method is adaptable to all kinds of pictures with absolute reliability, and all sources of defects otherwise occurring in the developing of photographic negatives are thereby avoided. The new process has the further advantage that it suppresses or at least does not emphasize the exposure of the emulsion particles near the surface of the emulsion. It is well known that these emulsion regions receive the full exposure with blue light, which light however is absorbed by the yellowish emulsion as it penetrates to deeper emulsion strata. Hence, the new process obviates in many cases the use of yellow filter, during the exposure of the negative, suppressing the blue light rays. The time required for the developing process may vary between about 4 and about 14 hours, and it becomes possible in consequence thereof to leave the plates to be developed in the liquid without special care, and to submit them to the fixing treatment, when the operator is at leisure.

## Examples

|                                                                                                                                     |          |    |
|-------------------------------------------------------------------------------------------------------------------------------------|----------|----|
| 1. Distilled water-----                                                                                                             | 100 cc.  | 80 |
| Sodium-sulfite-----                                                                                                                 | 15 grs.  |    |
| OH<br>Glycine $C_6H_4$ NH.CH <sub>2</sub> .COOH (amido-<br>oxy-phenyl-acetic acid)-----                                             | 3 grs.   | 85 |
| Potassium-bromide-----                                                                                                              | 1 gr.    |    |
| 2. Distilled water-----                                                                                                             | 400 cc.  |    |
| Metol $(C_6H_4$ OH<br>NH.CH <sub>2</sub> ) <sub>2</sub> H <sub>2</sub> SO <sub>4</sub> (methyl<br>amido-phenol-sulphuric acid)----- | 6 grs.   | 90 |
| Sodium-sulfite-----                                                                                                                 | 60 grs.  |    |
| Potassium-bromide-----                                                                                                              | 0.6 grs. |    |

The figures given above show the contents of a concentrated or commercial developing solution. For the practical use this developer should be diluted, e. g. in relation of 1 cubic centimeter to 25 cubic centimeters water.

Development of photographic silver haloid emulsions in substantially horizontal position, in undisturbed, alkali free and highly diluted developer solutions, as above described, has the following effects. The highly diluted alkali free developer quickly penetrates the emulsion, upon which it has no initial tanning action, so that development begins uniformly throughout the emulsion. When the development progresses, bromine is gradually set free with the above described beneficial effect upon the high light portions. After some time the developer begins to

100  
95  
105  
110

tan the surface of the emulsion with the effect that an excessive blackening of the surface regions of the emulsion, corresponding to the blue exposure, is avoided, although the emulsion is 5 fully developed throughout its thickness. The retarded surface tanning, due to the high dilution and the lack of alkali, also prevents wandering of the bromine, which is kept back in the deeper regions, thereby enhancing the previously de- 10 scribed halo and overexposure suppressing effect and hindering the wandering of bromine which often causes clouds and veils. This effect makes it moreover unnecessary exactly to level the emulsion, an approximately horizontal position being 15 sufficient.

It should, of course, be understood that the invention is not restricted to these specific exemplifications, but that it may include other embodiments both as regards material and proportions, 20 except as otherwise stated in the appended claims.

I claim:—

1. Photographic developer for long-time-hori-  
zontal developing, comprising a solution of sub-  
stantially sixty grams sodium-sulfite, substan-  
tially six grams metol and six tenths gram of po-  
tassium-bromide in substantially four hundred  
cubic centimeters of water, and free from caustic  
alkaline additions. 80

2. A method for developing photographic sil-  
ver haloid emulsions which comprises placing the  
emulsion support with the emulsion facing up-  
wardly and approximately horizontal into an  
aqueous solution of metol or glycine developing  
agent at a concentration of less than approxi-  
mately one quarter of one per cent, and not less  
than approximately one sixteenth of one per cent,  
containing water soluble sulfite but being sub-  
stantially free from alkali, and retaining the  
emulsion in said solution substantially undis-  
turbed several hours until fully developed. 85  
90  
95

FRITZ J. HEPNER.

25

100

30

105

35

110

40

115

45

120

50

125

55

130

60

135

65

140

70

145

75

150